

# UNITED STATES PATENT OFFICE.

JOHN H. LEWIS, OF JOPLIN, MISSOURI.

## COMPOSITION OF MATTER FOR REPAIR OF PNEUMATIC TIRES.

961,144.

No Drawing.

Specification of Letters Patent. Patented June 14, 1910.

Application filed August 19, 1909. Serial No. 513,668.

To all whom it may concern:

Be it known that I, JOHN H. LEWIS, a citizen of the United States, residing at Joplin, in the county of Jasper and State of Missouri, have discovered a new and useful composition of matter to be used for the treatment of any and all kinds of pneumatic tires to prevent the escape of the air in case they are punctured, of which the following is a specification.

My composition consists of the following ingredients, combined in the proportions stated, viz:—

|             |                 |
|-------------|-----------------|
| Ribbon glue | 38 pounds       |
| Water       | 1½ gallons      |
| Molasses    | 1 gallon 1 pint |
| Linseed oil | 5 pints         |

Dissolve the glue in the water in a steam jacket kettle until the glue is thoroughly dissolved and the water evaporates, then add the molasses and boil one hour, then add the linseed oil and continue boiling under a steam pressure of 80 to 100 pounds until a thick dark jelly compound is obtained, then remove from the kettle and cool. By the union of this compound in this manner we obtain the first chemical change.

To prepare the tire for treatment remove the valve stem and wash out the inner tube with gasolene to remove the soapstone and other foreign substances.

Weigh out the amount of compound necessary for the treatment of the tire and remelt in the steam jacket kettle and add the following heat resisting agents, which consist of:—

|                                              |                  |
|----------------------------------------------|------------------|
| Chrome alum                                  | 5 oz. 100 grains |
| Bichromate potash                            | 4 " 330 "        |
| Water sufficient to make twenty-five ounces. |                  |

To one pound of the compound add one-half ounce of the above, previously dissolved in hot water and stir; when thoroughly mixed transfer to a pump and force into the inner tube while hot through the valve stem opening; distribute equally in the tube by hand or the use of a roller, replace the valve stem and inflate with air, then place on a revolving drum and keep in motion 4 or 5 hours to throw the compound to the tread of the tire and to cool it. By combining the heat resisting agents in this manner we get the second chemical change.

By the treatment of tires with this compound they do not collapse and become useless for the reason that as soon as the tire is punctured the compound reunites and prevents the escape of the air.

I claim:

1. The hereinbefore described composition of matter consisting of ribbon glue, water, molasses, linseed oil, chrome alum, and bichromate potash, substantially as described and for the purpose specified.

2. The herein - described composition of matter for the treatment of pneumatic tires to prevent the escape of air when punctured consisting of ribbon glue 38 pounds, water 1½ gallons, molasses 1 gallon and 1 pint, linseed oil 5 pints, chrome alum 5 oz. 100 gr., bichromate potash 4 oz. 330 gr., water sufficient to make 25 ounces, substantially as described.

JOHN H. LEWIS.

Witnesses:

W. E. LEWIS,  
J. W. OGDEN.